

July 18, 1939.

A. LESAGE

2,166,634

PROCESS FOR MAKING ENGINE CYLINDERS WITH AN INNER LINING

Filed Feb. 17, 1938



INVENTOR

*Alfred Lesage*

BY

*Dean, Furbush & French*  
ATTORNEYS

## UNITED STATES PATENT OFFICE

2,166,634

PROCESS FOR MAKING ENGINE CYLINDERS  
WITH AN INNER LINING

Alfred Lesage, Schweißfurt, Germany

Application February 17, 1938, Serial No. 190,960  
In Germany February 15, 1937

1 Claim. (Cl. 22—203)

This invention relates to the cylinder of internal combustion engines and more particularly to cylinders having an internal surface layer of a harder metal than the cylinder, this lining being devised to form the slide way of the piston reciprocated in the cylinder.

An object of this invention is the method for making the liner in an easy, effective and cheap way.

10 In lining a casting of light-alloy containing a considerable percentage of aluminium with a melted harder metal or alloy having a higher melting point with the aim of obtaining an uniform and continuous thin layer the drawback often arises that the alloy with the lower melting point is liquefied as the heat cannot be removed quickly enough so that the two layers form a new alloy uniform in its hardness and resistance to wearing out, or the harder metal will enter the 20 light-metal to an uncontrollable extent thereby generating further inconveniences.

The new objects will be attained by a method allowing the lining operation to be well and continuously regulated by the gradual formation of 25 the liner. It has been found that a thin jet of the harder metal when applied to the inside surface of a light-alloy cylinder while advancing on the same in a lengthwise direction and peripherally, viz, along a helical line, will produce a metallic layer of uniform depth because it cools down more quickly. The thinner the jet of molten metal, the more uniform the layer produced, especially when being pressed against and distributed on the inside surface of the cylinder 35 by centrifugal force.

With the aid of the method according to the present invention it is possible to apply such a thin metal jet in the form of metallic threads narrowly juxtaposed on the inside surface of a cylinder and to cause the said threads to combine into a continuous layer which firmly adheres to the said cylinder.

To this end a rapidly rotated pouring funnel containing the liquid metal and the bottom end 45 of which is provided with a small outlet nozzle is introduced into the cylinder which is displaced at a suitable speed along its center line by mechanically driven means. Under the pressure resulting from gravity the metal flows out as a thin jet against the wall of the cylinder in a helical line. The pressure may be increased by a pressure fluid acting upon the contents of the funnel. The jet may also be applied along a helical line when there is imparted to the funnel a 55 movement in a lengthwise direction and a rapid

rotation, in which case the centrifugal force causes the liquid metal to more strongly adhere to the cylinder wall. The funnel may also be stationary while the cylinder at the same time has imparted thereto the said longitudinal and 5 rotary movements in which case the centrifugal force acting on the metal flowing into the cylinder will result in the layer applied being distributed more uniformly and smoothed accordingly. Also the funnel and the cylinder may be 10 rotated simultaneously, and in general the relative rotation and rectilinear displacement may be distributed between the funnel and the cylinder in any suitable way and proportion.

The accompanying drawing, forming a part of 15 this specification, by way of example shows an embodiment of the present invention, representing a device intended for producing the slide surface for the piston of a light-alloy engine cylinder, the figure representing a vertical section 20 along the center line of the said device.

For the production of the harder inside layer the cylinder is fastened to a carrier having the form of a disk 3 which is arranged at the top end of a vertical hollow spindle 4 and rotatably 25 mounted in bearings 5. By means of a pulley 6 fixed on the said spindle 4 and a belt 7 or of a similar driving appliance the spindle 4 may be rotated. Within this spindle there is revolubly mounted a shaft 8 carrying a pouring funnel 9 30 at its upper end which funnel is provided with a slanting outlet spout 10. The lower end of the said shaft 8 carries a pulley 12 which may be driven by a belt 13. The lower end of the spindle 4 is engaged by a sliding ring or a roller fork 35 14 which may be reciprocated in a vertical direction by means of a lever 15 or another suitable driving member in order to raise and lower the spindle 4. The carrier 3 is preferably provided with apertures 16 through which dropping molten 40 metal, if any, is thrown into the cup 17 where it collects.

The device is made use of in the following way: The liquid metal to be applied to the inside surface of the engine cylinder 18 is put into the 45 funnel 9 rotated by the driving means 12, 13 and then flows through the outlet 10 against the inside wall of the cylinder 18 while the same is at the same time raised by the appliance 14, 15 so that the liquid metal being poured is applied to 50 the cylinder wall in helical lines placed narrowly side by side. If a rapid rotation at the same time is imparted to the cylinder by the transmission means 6, 7 the harder metal applied thereto is pressed against the cylinder wall so 55

as to effect a partial fusion of the light metal of the cylinder having a lower melting point so that a connection free from joints and affording a highly satisfactory conductivity for heat will be obtained. By the centrifugal force the juxtaposed helical threads of the molten harder metal will also at once be pressed against one another and combined into a layer uniformly cohering and having about the same thickness throughout. In this way it is possible to produce a comparatively thin layer on the inside wall of the cylinder which layer will by the partial fusion of the metal thereof not only strongly adhere but also cool down so quickly that the cylinder itself will comprise several concentrical layers of different metals or alloys with distinct degrees of hardness. By providing the cylinder with heat radiating flanges 19, the temperature of the cylinder during the admission of the molten metal to form the liner may be readily maintained within such a range that the molten metal will rapidly solidify, the molten metal will not unduly melt the cylinder and will not be so instantaneously chilled as to prevent the desired partial melting and the formation of the bonding alloy.

The relative angular and axial displacements of both the cylinder and the funnel may be chosen in different manners according to the particular conditions prevailing so that a differential effect is obtained which causes the jet of liquid metal to strike the cylinder wall under an increased pressure. The funnel may be filled up to a definite level from the very start or be filled continuously, also a pressure fluid may be caused to act upon the contents of the said funnel.

When the process is being carried out, heat may be supplied or carried off so that the tem-

perature required for the application of the internal liner may be controlled at will.

The material to be used for the slide surface on which the piston runs may be a harder alloy melting at a higher temperature or a hard metal such as cast iron, steel, etc.

In case the inside layer is iron or steel the aluminium is preferably protected from burning, by an atmosphere of an inert gas, such as carbonic acid, being formed within and around the cylinder, which gas may at the same time also act as a cooling agent.

I claim:

The method of making an internal combustion cylinder with a light metal jacket having radiating fins and a lining of metal of substantially greater hardness and of substantially higher melting point, which comprises the steps of rotating a vertically disposed jacket, projecting a jet of the molten harder metal within and radially of said cylinder jacket, and against the inner periphery of the latter, effecting relative rotation of said jet and said cylinder, and continuously moving said jet axially of said cylinder, said jet being so fine that the metal therefrom solidifies quickly on the inner surface of the cylinder as a helical strip, and fuses only the inner surface portion of the cylinder jacket on which it is projected, to form a thin intermediate layer alloyed from said light metal and said harder metal, said jacket being rotated at such high speed, that adjacent turns of said helical strip are levelled off by centrifugal action to form a comparatively smooth substantially uniform continuous lining on said jacket under the cooling effected by radiation from said fins.

ALFRED LESAGE.